

## UNITED STATES PATENT OFFICE

1,991,410

PROCESS FOR CRYSTALLIZING BORAX  
FROM SOLUTIONSAlfred Newman, Long Beach, Calif., assignor to  
Pacific Coast Borax Company, a corporation of  
NevadaNo Drawing. Application July 30, 1932,  
Serial No. 627,133

6 Claims. (Cl. 23—59)

This invention has to do in a general way with the art of crystallization, and is more particularly related to the production of borax crystals from agitated aqueous solutions of borax.

5 It is well known to those familiar with the art, that if any aqueous solution of borax, which, by way of illustration, may contain 20 to 30% crystal borax in solution, is placed in a tank and is agitated in any suitable manner and rapidly cooled by any suitable means, such as contact with pipe coils through which a refrigerant, cooler than the borax liquid, is flowing, or by rapidly evaporating the water from the borax solution in a so-called vacuum cooler, the borax 10 crystals which precipitate from the solution are chiefly aggregates of small crystals, the individual particles having no definite form or shape. For convenience I define such crystals as type one.

15 Being of irregular shape the crystals readily cohere and upon packing the mass of crystals often becomes compact and hard and thus as commonly defined becomes "caked". Although borax crystals formed in this way are adapted for many uses it has been found advantageous for 20 some purposes to form a crystalline borax, the individual particles of which are of definite crystal form with distinct crystal faces characteristic of borax or  $Na_2B_4O_7 \cdot 10H_2O$ . For convenience I define such crystals as type two. Such 25 crystals, on account of their definite crystal form and distinct crystal faces, do not cohere or cake to the same degree as crystals of type one.

30 The trade having come to demand larger crystals it has been found desirable to produce by rapid cooling crystalline borax of a size larger than type one. It has been found that the type 35 one crystals hitherto produced by rapid cooling have approximately the following mesh:—

| 40 | Tyler mesh | Cumulative percent | Tyler mesh | Cumulative percent |
|----|------------|--------------------|------------|--------------------|
|    | 14         | 0.30               | 65         | 79.27              |
|    | 20         | 3.53               | 100        | 86.79              |
|    | 28         | 30.83              | 150        | 91.52              |
| 45 | 35         | 57.15              | 200        | 94.82              |
|    | 48         | 70.40              | —200       | 100.00             |

50 By the process herein described it has been found possible to produce crystals of type two having the following mesh:

| 55 | Tyler standard mesh | Cumulative percent | Tyler standard mesh | Cumulative percent |
|----|---------------------|--------------------|---------------------|--------------------|
|    | 10                  | .00                | 65                  | 88.24              |
|    | 14                  | 7.64               | 100                 | 93.74              |
|    | 20                  | 29.74              | 150                 | 98.24              |
|    | 28                  | 50.74              | 200                 | 99.74              |
|    | 35                  | 68.84              | —200                | 100.00             |
|    | 48                  | 73.84              |                     |                    |

The production of borax crystals of type two has hitherto been accomplished, first by very slow cooling of the borax solution, and second, by adding a small amount of soap, fatty acid, or other emulsion colloid of similar nature to the hot borax solution either prior to or during the step of rapid cooling and agitation. 5

The process of slow cooling obviously has marked disadvantages in the commercial process, since the time, from 6 to 7 days and equipment required for the production of a given amount of this type of borax is much greater than that which is necessary in a process that can be carried out by rapid cooling, say from 4 to 5 hours. The use of soap, fatty acid, or other emulsion 10 colloids often results in a quantity of the agent being entrained or entangled in the borax crystal. This quantity is sufficient to yield a discolored glass when the borax is fused, and when the borax is placed in warm water and the mixture 15 shaken the quantity is sufficient to produce a foam or lather similar to that when soap is added to warm water.

20 It is a primary object of my invention to produce borax crystals of type two and at the same time to avoid the undesirable results noted above. I have discovered that the object contemplated by my invention can be attained simply by seeding 25 a hot borax solution with a suitable quantity of borax crystals formed by the process of slow cooling another hot borax solution. It is preferable that the borax used as seed crystals be deposited from solution without agitation. By slow cooling 30 I refer to the type of process first enumerated above in which the hot borax solution is cooled merely by radiation to the atmosphere over a 35 substantial period of time. As pointed out above, the borax crystals formed by such a cooling process are of well defined crystalline form and shape and I have discovered that they have the 40 peculiar property, when added as seed crystals to another hot borax solution, of causing the crystals formed from the latter solution to also be of well defined crystal form and shape with distinct 45 crystal faces. This property seems to be peculiar to the crystals formed by the slow cooling process, and the fact is of particular value in that the 50 seeded solution can be rapidly cooled and agitated during crystallization without in any way interfering with the formation of the individual crystals.

The following example is given for the purpose 55 of more clearly illustrating the process contemplated by my invention. First, four thousand gallons, of hot aqueous solution of borax containing, say thirty per cent crystal borax, placed in a tank and allowed to cool by radiation of heat into the atmosphere for a period of six days. This time may be greater or less within certain limits without in any way affecting the results of the 60

process. The crystal borax thus formed is separated from the liquor and the crystals are crushed to a suitable size for use as seeds. I have found that the best results are obtained if the seed crystals are larger than what will pass a sixty-five mesh Tyler standard screen, or a screen having an opening of .0082 inch.

After a suitable quantity of these seed crystals has been prepared, in the manner described above, another suitable quantity, say four thousand gallons of hot aqueous solution of borax of approximately 185° F., containing, say twenty-eight per cent crystal borax, is placed in a tank, agitated, and rapidly cooled in any suitable manner until a temperature of substantially 135° F. has been reached. At this time a quantity, say seven hundred pounds of seed crystals, formed and sized as above described is added to the solution, the agitation and the cooling of the liquor being continued without interruption. From this point on the borax crystallizes quickly and the crystals formed are chiefly of definite crystal form with distinct crystal faces. The size of the crystals, of course, can be varied within certain limits by controlling the time over which the agitation and cooling takes place.

It has been found that proceeding in the above described manner crystals of the aforementioned characteristics are produced.

I have found that the mother liquor can be removed much more easily from crystals formed in the process contemplated by this invention than from the aggregation type of crystals ordinarily produced by rapid cooling a hot borax solution.

As a further advantage of producing larger size crystals, a given weight of the material when packed for shipment, occupies a volume of approximately eighty percent the volume occupied by the same weight of borax of the aggregation crystal type. My process, therefore, has the advantage of reducing the cost of production, (as compared with borax produced by the "slow cooling" process) reducing the cost of packing and shipping, (as compared with the "aggregate type" of crystal) and supplying to the trade crystals of borax which do not readily cake, and of a size suitably larger.

It will be noted from the foregoing description that I have used four thousand gallons as the quantity of solution from which the seed crystals are prepared and have also referred to four thousand gallons as the quantity of solution which is rapidly cooled. It is to be understood of course that the quantity of seed crystals added to the second solution is a comparatively small percentage of the total quantity of seed crystals produced during the slow cooling step.

It is to be understood that the term "concentrated solution" as used herein has reference to a borax solution of a temperature and concentration suitable for seeding without dissolving the seed crystals.

It is to be understood that, while I have herein referred to one preferred method of practicing this process, the invention is not limited by the precise terms of the foregoing description but includes within its scope whatever changes fairly come within the spirit of the appended claims. 5

I claim as my invention:

1. A process of crystallizing borax of definite crystal form and with distinct crystal faces from aqueous solution which comprises slow cooling 10 a hot aqueous solution of borax to crystallize borax therefrom; pulverizing and screening borax crystals thus obtained to a fineness such that it will be retained on a screen of .00082 inch opening; seeding a second hot concentrated solution 15 with the pulverized crystals; and rapidly cooling the second solution.

2. A process of crystallizing borax of definite crystal form and with distinct crystal faces from aqueous solution which comprises slow cooling 20 a hot aqueous solution of borax to crystallize borax therefrom; pulverizing and screening the borax crystals thus obtained to a fineness such that it will be retained on a screen of .0082 inch opening; seeding a second hot concentrated so- 25 lution with the pulverized crystals; and rapidly cooling the second solution with agitation.

3. A process of crystallizing borax of definite form with distinct crystal faces from a concentrated aqueous solution which comprises rapidly 30 cooling said solution and seeding the same with borax crystals obtained by slow cooling another borax solution, said seed crystals being of a size such that they will be retained on a screen having an opening of .0082 inch. 35

4. A process of crystallizing borax of definite crystal form with distinct crystal faces from a concentrated aqueous solution which comprises rapidly cooling said solution and seeding the same with borax crystals obtained by slow cooling 40 another borax solution, said seed crystals being of a size such that they will produce particles of well defined crystalline form and shape.

5. A process of crystallizing borax of definite form with distinct crystal faces from a concentrated aqueous solution which comprises rapidly 45 cooling and agitating said solution and seeding the same with borax crystals obtained by slow cooling another borax solution, said seed crystals being of a size such that they will be retained on a screen having an opening of .0082 inch. 50

6. A process of crystallizing borax of definite crystal form with distinct crystal faces from a concentrated aqueous solution which comprises rapidly cooling and agitating said solution and seeding the same with borax crystals obtained by slow cooling another borax solution, said seed crystals being of a size such that they will produce particles of well defined crystalline form and shape. 55

ALFRED NEWMAN. 60